

Aug. 13, 1946.

C. B. JACKSON

2,405,580

METHOD FOR PRODUCING ALKALI METAL OXIDES

Filed Dec. 14, 1940



BY

INVENTOR  
CAREY B. JACKSON  
*Frank E. Foste*  
ATTORNEY.

## UNITED STATES PATENT OFFICE

2,405,580

## METHOD FOR PRODUCING ALKALI METAL OXIDES

Carey B. Jackson, Forest Hills, Pa., assignor to  
Mine Safety Appliances Company, Pittsburgh,  
Pa.

Application December 14, 1940, Serial No. 370,159

10 Claims. (Cl. 23—184)

**1**  
This invention relates to a method of manufacture of oxides of metals, and more particularly, to a method and apparatus which may be used to produce uniformly and economically oxides of metals, such as potassium or sodium or a mixture thereof and the product of which is especially adaptable as an air purifying and oxygen evolving compound.

One of the methods heretofore available for oxidizing these alkali metals to a high oxide state and which method has had some commercial value consists of a two-step or two-stage method of procedure. In this method, the pure metal is oxidized first to a composition approximating the metal monoxide and this is accomplished by subjecting the surface of the pure molten metal to an oxidizing atmosphere. The oxygen content of the fluid or atmosphere supplied is limited to less than 10 per cent because any greater amount would produce an explosive condition due to the mass involved and the vapor pressure of the metal. The reaction itself is sufficiently exothermic to carry the reaction to completion and this provides a source of danger if too much mass is involved at one time. The high oxide or peroxide, which in the case of potassium is potassium tetraoxide ( $K_2O_4$ ) and in the case of sodium is sodium peroxide ( $Na_2O_2$ ), is then formed from the monoxide by subjecting the surface of the molten metal monoxide to oxidizing fluid. This reaction is not sufficiently exothermic to carry on the reaction and heat must be supplied continuously. One of the principal difficulties in this method is the fact that the reaction takes place slowly and it is difficult to produce a uniform product. The motivating force in this method which would provide uniformity of composition in the reactive mass is the capillary movement of the materials and it is apparent that this is slow and very difficult to control. Furthermore, this method is obviously very expensive to perform in commercial quantities due to the extensive equipment required in subjecting the surface of the material to an oxidizing atmosphere in the two stages of the method, and, also, in performing the second stage of the process, a large amount of heat must be continuously added to the mass to oxidize the metal to the highest available oxide.

In order to expedite this type of oxidizing procedure, it has been suggested to supply the molten metal in the form of thin layers and then subject these layers to the oxidizing atmosphere. Such procedure would, no doubt, improve the uniformity of the composition prepared, but a great

amount of time is still needed to complete the reaction and it necessitates the use of considerable equipment if the product is to be manufactured in commercial quantities.

**2**  
The physical characteristics of the resulting product of this general method is dense and hard and unsuitable for use in respiratory apparatus and no treatment has been found which will make the product of a nature that makes it suitable for this purpose. In some instances, the product formed is so hard as to dissolve only slowly in water. An air purifying composition, in order to be useful in respiratory apparatus must be of a porous nature or have such characteristics that it is instantly reactive with respired air by being penetrable by carbon dioxide and water to absorb carbon dioxide and to evolve oxygen to replace to some extent the oxygen consumed.

The principal object of this invention is to provide a method of forming an oxide of a metal and an apparatus for performing the method which is continuous, simple in operation, inexpensive and rapid in performance and commercially practicable and which is adaptable to produce potassium or sodium peroxide or a mixture thereof of uniform composition having definite physical characteristics rendering the product adaptable as an air purifying composition.

The method of my invention employs the treatment of molten metal which is to be reasonably pure, or at least not containing any impurities which would interfere with the process or prevent its being used for the purpose intended. The molten metal is made to flow and in an atomized state to form a stream of small or minute particles and this stream is then subjected to an oxidizing atmosphere. This atomization step renders the metal increasingly reactive and sufficiently so that a substantially uniform oxidized product is produced in a rapid and inexpensive manner. In carrying out the method for producing alkali peroxides, such as potassium peroxide, a small stream of molten metal is directed into a flow of fluid having an oxygen content of at least 13 per cent by volume and preferably not more than 35 per cent. Within these limits of oxygen content, the method can be carried on to the best advantage relative to the rate of production, uniformity and protection of apparatus. Since the constituency of ordinary atmosphere is within the designated limits, it is suitable for the practice of this method. By introducing a stream of the molten metal into a flow of air, fine spherical-like particles or globules of material are formed and suspended in the flow, and an in-

stantaneous or at least immediate oxidation occurs to the metal and this is carried directly and quickly to the highest state of oxidation of the metal. The oxygen content in air is ample to oxidize the metal to the desired state for metals like potassium provided sufficient volume is supplied for mixing with the metal in its atomized state. The fact that the overall reaction is exothermic in these oxidation reactions and to a relatively large value, sufficient heat is available to carry the reaction of all the metal to completion by this continuous process.

It was thought that any method based upon the atomization of such reactive metal as potassium and sodium would be dangerous in that the mixture of the metal with atmosphere would be dangerously explosive and thus any such hazards would render the method impractical for commercial purposes. It has been found that by controlling the oxygen content within the limits set forth above, any such dangers are eliminated sufficiently provided some care is taken in the practice of the method and it can be and is being performed on a commercial scale, with inexpensive apparatus and at a low cost of operation.

In order to prevent the oxide from becoming hard and of a high density, it is cooled quickly by the flow of air and reduced below the fusion temperature of the oxide. Ordinarily, atomized molten metal when oxidized appears to burst open or explode the spherical shape or globule type of particles, and when cooled it reassumes this globule shape due to the surface tension of the material. This immediate cooling of the reacted material appears to cause it to remain in the bursted condition, it being what might be termed frozen in this condition, and this physical condition is of an aborescent, or fluffy, nature in structure and because of this property is especially adaptable for respiration apparatus.

For the purpose of aiding in giving a full and complete description of the method, an apparatus is illustrated and described which has been used for producing potassium tetra-oxide in commercial quantities. Referring to the drawing, the apparatus is simply a fluid spray device such as is used to apply paints or other coating on to surfaces and which has been found to be adaptable to discharge a thin or fine stream of metal, this being controlled by an adjustment which forms a part of the device. The stream is diverted into an air flow which effects an atomization of the metal.

The device is made of a metal material which is not affected by the temperatures involved in this method and comprises a housing 1 having a passage 3 and a passage 4. These passages are connected to suitable tubes, which in turn are connected to a source of oxidizing fluid and to the molten metal, respectively. A vented receptacle 5 contains the molten metal and a tube 4a connected to the passage 4 is inserted therein. An opening 7 is provided in the housing for the passage 4, while an opening 6 which is aligned with the opening 7 is provided for the passage 3.

The oxidizing fluid under pressure is introduced into the housing through the passage and completely encircles the passage 4 containing the molten metal and by being discharged at a relatively high velocity at the opening 6 and over the opening 7 is effective to draw the molten metal up into the passage and against a needle adjustment 9. This adjustment controls the discharge of the metal particles from the device and by such the metal is discharged from the

device in a thin or fine stream of the molten metal and which when being directed into the fluid flow is dispersed so as to form finely divided particles of the molten metal, which operation will be hereinafter described as atomization. For the purpose of collecting the oxidized metal, a receiving chamber 8 is directly connected to the atomizing device and it has a vent 8a connected to the atmosphere so that an ordinary atmospheric condition exists within the chamber and a discharge 8b is provided in its lower extremity. The operation of this device is not described in detail nor is the apparatus since it is a device well known in the art and its principle of operation is likewise well known.

In the use of such a device for the practice of my method, the molten metal contained in the receptacle 5 is drawn into the passage 4 of the housing proper by the flow of oxidizing fluid, introduced into the passage 3, over the opening of the passage 4 or in such relation that the molten metal is discharged from the device in a small stream readily dispersable and into the stream of oxidizing fluid producing the suction and carrying the formed metal particles or atomized stream of metal into the receiving chamber 8. The metal particles are intimately mixed with the oxidizing fluid and because of this and the molten state of the metal as well as the heat evolved, an instant reaction of the metal and the fluid is caused to oxidize the metal completely to its highest state. No means or medium is required to initiate the reaction, since the molten metal particles in the oxidizing fluid flow are instantaneously reactive. The heat evolved also accelerates the reaction and the excess of oxygen present causes the oxidation to be rapidly carried to completion.

In employing this process in a commercial manner to produce potassium tetra-oxide, it being understood that any reference to peroxide is to be construed to mean the highest state of oxidation attainable and suitable for commercial use, the oxidizing fluid flow is produced by connecting the passage 3 of the housing to a source of ordinary atmosphere or air at a sufficiently high pressure. In one instance, which has proven to be a commercial application, the air is at about 20 pounds pressure and at a temperature of about 75° C. The potassium metal is heated to a molten state and maintained in this state during the performance of the method and is preferably at a temperature several degrees above its melting point. In any event, the temperature should be such that a slight reduction would not cause a solidification or any thickening of the molten metal and prevent its being readily and efficiently atomized or discharged in a stream atomized by impingement against a stream of air. For some purposes, it may be advisable to provide some form of an inert atmosphere over the surface of the metal contained in the receptacle 5 in order to prevent any contamination of the metal before it is introduced into the atomizing device.

By heating the compressed air to a temperature of about 75° C., the metal within the housing 1, or specifically within the passage 4, is maintained in a molten state while passing through the device. However, this function of the air is more or less ancillary because in using air for the practice of my method the oxygen of the air is the source supplied for oxidizing the potassium while the nitrogen of the air, inert to potassium or the formed oxide, cools the peroxide in a prescribed manner.

Theoretically, about 43 cubic feet of air is required to oxidize a pound of potassium to potassium tetra-oxide. Obviously, a continuous method of the type involved does not utilize fully the oxygen available, and for this purpose, as well as the amount needed to accomplish the high state of oxidation, a considerable excess of oxygen must be supplied. The other requirement in supplying an adequate rate of flow of air to accommodate a rate of flow of potassium and which constitutes an important feature of my invention is that the air of the flow must have sufficient cooling capacity to quickly cool or quench the peroxide as it is formed and to the extent that the temperature of the material is lowered below its fusion temperature.

In the formation of a pound of potassium peroxide, about 135 kilo calories are evolved. While this amount of heat represents a substantial amount, it is to be remembered that the fusion temperature of the oxide is considerably higher than the temperature of the molten metal and the weight of oxide formed is about 1.8 times the weight of the metal so that the amount of heat that must be absorbed to lower the temperature of the peroxide sufficiently does not necessitate any complete absorption of the heat evolved. On the other hand, air has a low specific heat and this property requires a flow several times the amount required for oxidation purposes. The temperature of the air supplied, unless serving as a medium of maintaining the metal in a molten state, should not be too low or some difficulty may be encountered in starting the reaction. However, ways and means can be provided for supplying heat in initiating the reaction and in maintaining the metal molten before being mixed with the air, so that the temperature of air depends mostly on the available supply. It has been found for commercial purposes that by supplying from 5 to 15 times the theoretical amount of air required for oxidation and at about 75° C. the air has sufficient cooling capacity to instantly lower the temperature of the formed peroxide below its fusion temperature.

In the application of my method, using the spray device illustrated, compressed and heated air enters the passage 3 of the atomizing device and is discharged into the receiving chamber 8, which is at atmospheric pressure, at a relative high velocity. This velocity moves past the opening 7 of the passage 4 in such a manner to draw the metal from the receptacle 5 into the air stream. To accommodate a flow of potassium of about 5 pounds per hour, an adequate flow of air is provided by discharging air under a pressure of 20 pounds into the receiving chamber 8 through six openings each having an opening of an area equal to that through which the potassium is drawn. The opening for the molten potassium is about  $\frac{1}{16}$ " in diameter and is controlled by the needle adjustment, so that the proper proportions of air and potassium can be established by varying the flow of potassium.

Almost instantly at the point of mixture of the flow of air and molten potassium, the oxidizing reaction begins and continues at a rapid rate and is carried on with the reacting mass for a very short period of time, such as may transpire in movement of the mass only a few inches beyond the outlet opening of the device. The oxygen content of the fluid determines the rapidity of the oxidation and it has been found that by using a flow of fluid of about all oxygen that the oxidation starts at about the tip of the device and

the result was that due to the extreme rate of the reaction the heat given off melted the tip of the device and rendered it inoperative. A lesser oxygen content causes the oxidation to start adjacent the tip of the device and as the content is decreased the reaction starts farther distant from the tip until the amount of oxygen is insufficient to give complete oxidation. On this other extreme, a fluid having an oxygen content of about 8% by volume had a slightly delayed action in starting the reaction and when started it was prolonged and it was found that some unoxidized particles of metal appeared in the mass forming in the collecting chamber. Thus, while the limits of from 13% to 35% do not establish critical limits of the operativeness of the method, yet from a commercial standpoint a fluid having this oxygen content gives the best operating results in view of cost of performance of the method, deterioration to equipment and uniformity of product. This flow method of mixture and oxidation provides a continuous stream of reacting material. Sufficient collecting space should be provided into which the discharge from the device can be directed so that the air stream and suspended reacting mass are not obstructed but completely spent substantially before the walls of the confined space or chamber are encountered. The cooling of the peroxide to a temperature below its fusion temperature follows the oxidation and because of the velocity of the reacted mass and air and the movement of each relative to the other, the lowering of the temperature is actually what might be termed a quenching. Following the cooling, the oxide settles to the bottom of the chamber, as illustrated, and can be removed by means of the closure 8b. The product is uniform and of an arborescent physical structure which makes it instantly reactive with respiration air to absorb carbon dioxide and evolve oxygen.

It is apparent that the successful operation of this method is not dependent upon any specific set of conditions of operation except for the general requirements of providing the active metal in a molten state so that it may be readily and conveniently atomized and intimately mixed with a flow of oxidizing fluid and producing an intimate mixture of the fluid and atomized metal such as by directing one stream into the other. The fluid should have sufficient oxygen content to oxidize the metal in a manner depending upon the conditions present and the product desired and a content of inert material in the fluid to control the physical state of the product, as by setting the metal in its oxidized molten state by an instant cooling or quenching.

It is obvious that other means can be employed for atomizing the metal in a stream of oxidizing fluid. Also, while this invention has been described particularly in connection with the forming of a high oxide of potassium ( $K_2O_4$ ), the method can be employed equally as well for forming a high oxide of sodium as well as a high oxide of a substance comprising a mixture of sodium and potassium which would form a mixture of sodium and potassium peroxide. It has been found in oxidizing sodium that because it is less reactive as compared to potassium, this refers to the rate of reaction to which the sodium is oxidized to the desired state, some of the lesser oxides of the metal are produced unless the sodium is atomized to a more minute degree than the potassium and the rate of discharge of the sodium is compensated accordingly. The oxidation reaction is also exothermic and is sufficiently so to make the reaction spontaneous. Any heat

supplied is for the purpose of keeping the metal in a molten state at the time of discharge into the stream of oxidizing fluid. The heat in the molten metal is adequate to initiate the oxidation and the heat evolved by the reaction accelerates the rate.

In all cases of application of my method, the chemical properties of the selected metal must be considered in adapting my invention to the metal. The properties of the metal upon which the method depends are known and the adaptation of my method to the selected metal can be made by those skilled in the art. By proper control of the flow of the molten metal and the oxidizing fluid, the desired oxidation product can be produced. However, the metal to be oxidized must be such that it can be atomized in a molten state and intermixed in an oxidizing flow and which by atomization becomes sufficiently reactive within the apparent limits of the invention to form the desired oxidation product.

One of the conditions that appears to lessen the hazards that exist in treating the highly reactive alkali metals is the vacuum that is utilized in atomizing the molten metal. It is apparent that if a positive pressure sufficient to move the metal to the point of discharge and then discharge it at a sufficiently high velocity is applied to the metal and the metal under pressure introduced into a flow of oxidizing fluid that some conditions might be created for certain metals which would result in a very hazardous condition of operation. Consequently, this method of discharge of the metal is preferred although it is apparent that it is not indispensable in the practice of the method. This vacuum also eliminates any premature firing or ignition of the metal.

It is intended that this detailed description of my method as specifically applied to the oxidation of alkali metals, and particularly of potassium metal, discloses the principle involved and the exemplary apparatus by which the method can be carried on satisfactorily are what I now consider to be the best application of my invention, but it is intended that the invention be limited only by the scope of the appended claims.

I claim:

1. That method of making alkali metal oxide which comprises spraying molten alkali metal into a current of an atmosphere containing oxygen and a gas inert to said metal and thereby oxidizing the metal rapidly, and supplying said atmosphere in an amount such as to provide an excess of oxygen over that theoretically necessary for said oxidation and such, relative to its temperature, as to quench the oxide below its melting point substantially as rapidly as it is formed, and thereby producing the oxide in a fluffy and uniformly oxidized form of low apparent density.

2. A method according to claim 1, said atmosphere being heated prior to contact with said sprayed metal to a temperature to maintain said alkali metal molten during oxidation.

3. That method of making alkali metal peroxide which comprises atomizing molten alkali metal into a current of an atmosphere containing about 13 to about 35 per cent of oxygen and a gas inert to said metal and heated to a temperature to maintain said metal molten and thereby oxidizing the particles of metal rapidly to peroxide, and supplying said atmosphere in

an amount such as to provide an excess of oxygen over that theoretically necessary for said oxidation and such, relative to its temperature, as to quench the oxide below its melting point substantially as rapidly as it is formed, and thereby producing the peroxide in a fluffy and uniformly oxidized form of low apparent density and of high reactivity with exhaled air.

4. A method according to claim 3, said atmosphere being air.

5. That method of making alkali metal peroxide which comprises atomizing molten alkali metal at a temperature above but close to its melting point into a current of air heated to a temperature to maintain the metal particles molten and thereby rapidly oxidizing the metal particles to peroxide, and supplying said current of air in an amount such as to provide an excess of oxygen over that theoretically necessary for said oxidation and such, relative to its temperature, as to quench the oxide below its melting point substantially as rapidly as it is formed, and thereby producing the peroxide in a fluffy and uniformly oxidized form of low apparent density and of high reactivity with exhaled air.

6. A method of making potassium tetroxide according to claim 5, said metal being potassium, and the potassium and air being heated to about 75° C.

7. That method of making alkali metal peroxide which comprises providing a body of at least one metal of the group consisting of sodium and potassium in the molten state, continuously atomizing the molten metal with a stream of gas under pressure and containing from about 13 to about 35 per cent of oxygen and substantially all of the remainder inert to said metal, said gas being heated to a temperature to maintain said metal molten, and regulating said stream to provide an excess of oxygen over that theoretically necessary to convert said metal to the peroxide state and such, relative to its temperature, as to quench the peroxide below its melting point substantially as rapidly as it is formed, and thereby producing the peroxide in a fluffy and uniformly oxidized form of low apparent density and of high reactivity with exhaled air.

8. A method according to claim 7, said metal being postassium and said peroxide being potassium tetroxide.

9. A method according to claim 7, said metal being potassium, said peroxide being potassium tetroxide, and said current of air being supplied in an amount such as to provide from about 5 to about 15 times the amount of oxygen theoretically necessary for oxidizing the metal.

10. That method of making peroxide of metal of the group consisting of sodium and potassium which comprises spraying the molten metal in a current of an atmosphere of gas inert to the metal and containing oxygen into a chamber heated only by the heat liberated therefrom, supplying said atmosphere in an amount such as to provide oxygen in excess of that necessary for said oxidation and such, relative to its temperature, as to quench the peroxide formed below its melting point substantially as rapidly as it is formed, and thereby producing said oxide in a highly porous and reactive form of low apparent density.

CAREY B. JACKSON.